

June 17, 1930.

F. L. KELLER

1,764,633

METHOD OF MANUFACTURING DIES

Filed May 22, 1926



Inventor  
Frederick L. Keller  
by H. A. Hansen Atty.

## UNITED STATES PATENT OFFICE

FREDERICK LAWRENCE KELLER, OF CHICAGO, ILLINOIS, ASSIGNOR TO WESTERN ELECTRIC COMPANY, INCORPORATED, OF NEW YORK, N. Y., A CORPORATION OF NEW YORK

## METHOD OF MANUFACTURING DIES

Application filed May 22, 1926. Serial No. 110,847.

This invention relates to methods of manufacturing dies, and more particularly to methods of manufacturing blanking dies.

An object of the invention is to simplify 5 and improve the construction of dies and thereby reduce the amount of labor involved in the finishing of the openings in such dies.

The invention contemplates the swaging of the material of which a die is made, 10 around a mandrel and then withdrawing the mandrel to leave an opening corresponding to the shape of the mandrel. In accordance with one embodiment of the invention, the opening in the blanking die is made some- 15 what larger than required and the opening is then reduced to the proper size by subjecting the die to a high pressure causing a cold flow of the metal around the mandrel which is of the size required for the opening.

20 It is believed that a better understanding of the invention may be had by reference to the following description taken in conjunction with the accompanying drawing showing an apparatus by means of which the invention may be practiced, and in which

Fig. 1 is a fragmentary plan view of a die and mandrel associated with a yoke as they appear in the initial stage of the swaging process;

30 Fig. 2 is a fragmentary sectional view taken on the line 2—2 of Fig. 1 showing in addition portions of the ram and bed of a hydraulic press in position to press the die into the tapered bore of the yoke, and

35 Fig. 3 is a reduced plan view of the yoke and die.

Referring to the drawing in which similar reference characters represent the same parts in the various views, the numeral 6 40 designates a die member of the type used in punch presses for blanking variously shaped flat pieces such as are used extensively in telephone and other apparatus. The die member illustrated is designed for punching blanks for forming contact springs having the shape of the opening in the die.

In order that a punch press in which such dies are used may operate properly it is necessary that the outline of the opening in 50 the die element conform precisely to the out-

line of the punch. Heretofore it has been the practice in some cases to file the opening to its final size manually, involving a great amount of accurate and skilled labor since these parts are usually made of hard metals such as carbon tool steel. 55

According to the present invention, an opening 11 is made in the die member slightly larger than a mandrel 12 which consists of a rectangular base 4 and a shank 5 of hardened carbon tool steel. No special attention is paid to the size or the exactness of the outline of the opening in the die except that it be larger than the mandrel. The ideal condition is an opening ranging from 1/200 inch to 1/64 inch larger than the arbor. The opening is then reduced to the proper size by subjecting the die to a high lateral pressure which is produced by forcing the die down a tapered opening 9 of a yoke 7 of hardened carbon tool steel. The yoke has a grip 20 to facilitate handling it and a band 17 of sheet metal is provided about the exterior of the yoke to prevent the yoke from scattering if it should burst due to the high pressure. The die member 6 is turned about its outer periphery, with a beveled edge having a 3 degree angle which corresponds with the slope of the frusto-conical opening 9 of the yoke, and its size is such that its greatest diameter is equal to the greatest diameter of the opening in the yoke, therefore, when the die is placed in the yoke, its top surface will lie flush with the top surface of the yoke. 60 65 70 75 80 85

The upper part of the die has a reduced portion 15 since it has been found that when the die blank is made as a regular frustum there is a tendency for it to buckle and become distorted due to the fact that there is a contraction along the diameter. When the upper portion of the die is reduced as shown, this tendency is greatly minimized, since the space thus provided affords a place for the metal to flow. 90 95

When the die is placed in the yoke a spiral compression spring 14 holds the mandrel in position and as the die is forced down into the yoke by a ram 16 of a hydraulic 100

press of any suitable type (not shown) an immense lateral pressure is exerted on the die causing a cold flow of the metal around the arbor.

5 As an example in the process of producing a carbon tool steel die 5 inches in diameter, a yoke 7 of hardened carbon tool steel is placed upon a bed 18 of a hydraulic press. A coating of white lead and oil is applied to the inclined surface of the yoke and to the beveled edge of the die and a similar coating is applied to the mandrel and the walls of the opening in the die. The mandrel is then inserted in the die opening and 10 the die is positioned in the yoke and pressed down the tapered bore of the yoke about two inches under a pressure of approximately sixty-five tons. During this operation the thickness of the die increases about  $1/16$  inch 15 and the metal of the die is forced around the mandrel giving the required shape and size to the opening. After the pressure is removed, the die is forced out of the yoke by any suitable means and the mandrel is 20 removed completing the die.

It will be understood that the embodiment of the invention herein described and illustrated is merely a useful and convenient form of the invention, which is capable of 25 many other modifications without departing from the spirit and scope of the invention.

What is claimed is:

1. A method of making a die, which consists of forming a circular beveled edge 30 around a die blank, reducing the periphery of the die blank at its greatest diameter to prevent buckling, making an opening in the die blank and reducing the size of the opening by exerting a pressure on the beveled edge of the die blank to force the material around a member of the desired shape.

2. A method of making a die, which consists of making an opening in the die blank differing from the required opening, reducing 45 the periphery of the die blank to prevent buckling, and altering the opening in the die blank by causing a cold flow of the material around the opening.

3. A method of making a die having a 50 plane upper and lower surface, which consists in forming a frusto-conical disk with a reduced portion at its greatest diameter to prevent buckling, making an opening of predetermined size through the body of the 55 disk, placing a member of the desired shape within the opening, and reducing the opening to a shape determined by the member by causing the material of the disk to flow laterally into engagement with the member by 60 exerting a radially inward pressure on the blank.

4. A method of making a die, which consists in forming a disk having a plane surface, shaping the sides of the disk to a frusto-conical shape, forming a reduced portion at

the base of the frusto-conical section, making an opening through the body of the disk, placing a member of the desired shape in the opening, and causing the material of the disk to move substantially in planes parallel to the plane surface of the disk by exerting a radially inward pressure thereon to change the opening to the shape of the member.

In witness whereof I hereunto subscribe my name this 7th day of May, A. D. 1926.

FREDERICK LAWRENCE KELLER.

70

75

80

85

90

95

100

105

110

115

120

125

130